

June 29, 1954

R. L. MITCHELL

2,682,536

AGING ALKALI CELLULOSE

Filed May 22, 1952



INVENTOR

Reid Logan Mitchell

BY

Dennis, Almonds, Motley, Barrow and Taylor

ATTORNEYS

## UNITED STATES PATENT OFFICE

2,682,536

## AGING ALKALI CELLULOSE

Reid Logan Mitchell, Shelton, Wash., assignor to  
 Rayonier Incorporated, Shelton, Wash., a corporation of Delaware

Application May 22, 1952, Serial No. 289,259

1 Claim. (Cl. 260—233)

**1**  
 This invention relates to the viscose process and has for its object the provision of certain improvements in the aging of the alkali cellulose for use in the manufacture of viscose. More particularly, the invention is concerned with the use of cobalt as a catalyst for the depolymerization of the cellulose to decrease its viscosity (commonly called "aging"). In accordance with the invention, a critically small amount of cobalt, preferably correlated to the alpha-cellulose content of the pulp, is incorporated in the pulp to control aging.

Various suggestions have been made heretofore to add cobalt to wood pulp and also to alkali cellulose to diminish the aging time. However, the use of cobalt for this purpose has not been satisfactory due to the fickle and unpredictable results. In fact, cobalt has been regarded as objectionable because it was not understood that an amount of cobalt that would give a desired aging effect in one pulp would give an entirely different aging effect in a pulp having a different alpha-cellulose content. It was further not foreseeable, from the experience in using other metals such as iron or manganese, that such a small quantity of cobalt would have such a pronounced effect on aging.

The invention is based on my discovery of a critical relationship between the alpha-cellulose content of the pulp, the per-cent reduction of aging, and the amount of cobalt incorporated in the pulp. One of the surprising aspects of the discovery is that such extremely small amounts of cobalt exercise such pronounced, and different, effects on the aging of the alkali cellulose. In accordance with the invention, such an amount of cobalt, suitably correlated to the alpha-cellulose content of the pulp, is incorporated in the pulp to effect a predetermined and desired reduction in the aging period of the alkali cellulose. I have found that less than 10 p. p. m. (parts per million) of cobalt based on the bone dry weight of the pulp is an amount sufficient to give practically any desired control over aging. However, even with amounts less than this small maximum amount, care must be taken not to use such an excessive amount as to cause undue degradation of the cellulose. For most aging requirements, satisfactory results are attained with less than 5 p. p. m. of cobalt, suitably correlated to the alpha-cellulose content of the pulp and the aging effect sought. With some pulps, very effective reduction in the aging time can be achieved with less than 1 p. p. m. of cobalt, but it is generally advantageous

**2**  
 in the interest of uniformity, due to the difficulty in dispensing such small amounts, to incorporate at least 1 p. p. m. of cobalt in the alkali cellulose pulp. The cobalt may be added to the pulp or to any material used in the preparation of the alkali cellulose, as for example, to the wood pulp, to the caustic soda or to a mixture of these when in a slurry. The cobalt is preferably added in the form of a water soluble compound such as cobaltous sulfate, nitrate, or chloride, etc. The references herein to the amount of cobalt in p. p. m. refer to the contained elemental cobalt and not to the compound, and the amounts of cellulose are on the basis of bone dry cellulose.

The accompanying coordinate diagram illustrates the critical effect of cobalt on the aging of alkali cellulose formed of pulps containing different percentages of alpha-cellulose such as are used for conversion to alkali cellulose in the viscose process.

Alpha cellulose content is one of the most commonly used measures of pulp purity; among other things it (1) reflects, particularly for wood pulps, the amount of alkali used in refining which in turn is related to degree of mercerization and potential ease of depolymerization of the finished pulp, and (2) parallels the absorptive affinity and cleavage sensitivity of the pulp to cobalt.

The term alkali cellulose "aging" or "aging requirement" as used herein refers to the period of storage subsequent to shredding and prior to xanthation in which sufficient depolymerization is accomplished so that the resultant viscose will have normal spinning viscosity.

It will be noted by reference to the chart that, say, 0.25 p. p. m. of cobalt will effect a 75% reduction in the aging of 98% alpha-cellulose, but only a 50% reduction in aging of 95% alpha-cellulose. It will be noted also by reference to the 75% reduction curve that a 92% alpha-cellulose requires 2 p. p. m., while a 97% alpha-cellulose requires but 0.3 p. p. m. to reduce the aging period to the same amount. Similar other wholly unpredictable comparative effects are clearly evident. In accordance with the preferred and most advantageous embodiment of the invention, I incorporate in the alkali cellulose the amount of cobalt within the shaded area of the chart, preferably correlated with the alpha-cellulose content of the pulp and the per-cent of aging desired.

The cobalt may be incorporated in the reacting materials in any suitable way provided it

is present in the alkali cellulose, and especially where a shredding operation is used because additional beneficial results will occur in shredding. However, there is an important advantage to be gained in the way of the uniformity of results by introducing the cobalt in the pulp since cobalt is tenaciously adsorbed and stripped from caustic soda steeping liquor by cellulose, and it is difficult in commercial operation to control satisfactorily the amount of cobalt in the steeped alkali cellulose by dissolving cobalt salts in the steeping liquor. While the cobalt thus added may be effective in lowering viscosity, the important thing is not merely to lower viscosity but to lower it in a continuously uniform manner.

The cobalt additions may be applied to the cellulose by any suitable method ensuring uniformity in the level of added cobalt. In one method of application I prefer to spray a dilute solution of cobalt sulfate onto the formed pulp sheet as it passes into the dryer on the pulp machine. In another method I prefer to apply a solution of cobalt sulfate at a uniform level as  $\frac{1}{4}$  inch strips along the machine direction of the formed pulp sheet, either while in the pulp dryer or later in the cutter used to cut rolls into sheets.

Since added cobalt in the extremely small amounts of 1-10 p. p. m. is not visible on the pulp sheet it is sometimes desirable to add a suitable dye to the cobalt treating solution in such amount (1 part dye to 1000 parts cobalt is sufficient for Victoria Green) as to label and identify the treated pulp.

The following examples illustrate methods carried out in accordance with the invention in the preparation of viscose from refined wood pulp in which DP refers to degree of polymerization:

#### Example I

A web of highly refined wood pulp (780 DP, 88% alpha-cellulose) was sprayed uniformly while entering the dryer of the pulp machine with a dilute solution of cobaltous sulfate in such amount as to add 2 p. p. m. cobalt based on bone dry pulp. This pulp was steeped in the customary manner in an equilibrium caustic soda steeping liquor containing 1.5% hemicellulose and 18.5% sodium hydroxide for 30 minutes at 30° C. The alkali cellulose sheets were then pressed to a press ratio of 2.70 and shredded for 1 hour at 30° C. The alkali cellulose crumb was aged for 15 hours at 30° C. It was then xanthated for 1½ hours using 31% CS<sub>2</sub> based on cellulose in alkali cellulose. The xanthate was mixed in a dissolver for 2 hours at 15° C. to give a viscose having the composition of 8.5% cellulose and 5.25% sodium hydroxide. After ripening for 24 hours at 20° C. the resulting viscose had a viscosity of 35 sec. falling-ball (5,300 centipoises) (300 DP) a salt index of 7.5 and gave a filtration plugging value of 1500 g./sq. cm. A sample of identical pulp but without the cobalt addition, processed in analogous manner, required 30 hours aging at 30° C. to give the same viscose viscosity. Viscose filtration for this latter pulp was 1400 g./sq. cm. Tensile and durability properties of films cast from the two viscoses were equivalent.

#### Example II

Sheets of cellulose pulp (780 DP, 88% alpha-cellulose) stripped with a solution of cobaltous sulfate in such manner as to contain 5 p. p. m. cobalt based on the bone dry weight of the pulp were steeped for 30 minutes at 30° C. in an equilibrium caustic soda liquor containing 1.5% hemi-

70

75

cellulose and 18.5% sodium hydroxide, pressed to 2.60 press ratio, shredded for 60 minutes at 30° C. aged for 24 hours at 30° C., xanthated for 1½ hours at 30° C. using 30% CS<sub>2</sub>, mixed for 2 hours at 15° C. to give a viscose containing 10% cellulose and 5% sodium hydroxide, then allowed to ripen for 24 hours at 20° C. The viscose had a viscosity of 35 sec. falling-ball (5,300 centipoises) (185 DP) a salt index of 6.5 and gave a filtration value of 1000. In the preparation of a similar viscose from pulp containing no added cobalt an aging time of 72 hours at 30° C. was required. Both viscoses had similar filterability and gave film of equivalent quality.

#### Example III

Sheets of a cellulose pulp (800 DP, 89% alpha-cellulose) containing 2 p. p. m. cobalt were steeped in a caustic soda steeping liquor containing 1.5% hemicellulose and 18.0% sodium hydroxide, pressed to 2.60 press ratio, shredded for 1 hour at 30° C., aged 18 hours at 30° C., xanthated for 1½ hours at 30° C. using 28% CS<sub>2</sub> based on the cellulose in alkali cellulose, mixed to give a viscose containing 8.5% cellulose and 4.0% sodium hydroxide, then ripened for 24 hours at 20° C. The viscose had a viscosity of 40 seconds falling-ball (6,000 centipoises) (285 DP) a salt index of 5.5 and a filtration value of 750. In the preparation of a similar viscose from identical pulp containing no added cobalt, the alkali cellulose aging requirement was 36 hours at 30° C.

#### Example IV

Sheets of a pulp (1150 DP, 95% alpha-cellulose) containing 0.5 p. p. m. added cobalt were steeped in a caustic soda steeping liquor containing 1.0% hemicellulose and 19.0% sodium hydroxide, pressed to a 2.50 press ratio, shredded for 1 hour at 30° C., aged for 10 hours at 30° C., xanthated for 2 hours at 30° C. using 34% CS<sub>2</sub>, mixed to give a viscose containing 7.5% cellulose and 6.5% sodium hydroxide, then ripened for 24 hours at 20° C. The viscose had a viscosity of 45 sec. falling-ball (6,700 centipoises) (400 DP) a salt index of 9.5 and a filtration value of 3500. In the preparation of a similar viscose from identical pulp containing no added cobalt, an aging time of 30 hours at 30° C. was required. The filtration value of the latter viscose was 3200. Tire cords prepared from the two viscoses had equivalent quality factor and fatigue life.

#### Example V

Sheets of pulp (1050 DP, 93% alpha-cellulose) were treated to contain 0.5 p. p. m. of added cobalt. The aging requirement was then equivalent to that for a 600 DP pulp although the actual DP was unchanged by the treatment.

#### Example VI

Sheets of pulp (2000 DP, 96.5% alpha-cellulose) were treated to contain 0.5 p. p. m. of added cobalt. It aged like a pulp of 1150 DP.

With 1 p. p. m. of added cobalt it aged like a pulp of 780 DP.

With 10 p. p. m. of added cobalt it aged like a pulp of 600 DP.

Various compounds of cobalt may be used. For reasons of economy and convenience in application, the water soluble inorganic cobalt compounds, such as cobaltous sulfate or nitrate, are very desirable.

*Example VII*

Pulp of 96% alpha, 1650 DP, treated to contain 1 p. p. m. cobalt added as a narrow strip (dyed green with Victoria Green, 0.001 p. p. m. on cellulose) was steeped in equilibrium steeping liquor containing 1.0% hemicellulose and 18.5% sodium hydroxide for 1 hour at 25° C., pressed to 2.60 ratio, shredded 1 hour at 30° C., aged for 7 hours at 30° C., xanthated for 2 hours at 30° C. using 34% CS<sub>2</sub>, mixed to give a viscose containing 7.5% cellulose and 6.5% sodium hydroxide, then ripened for 24 hours at 20° C. The viscose had a viscosity of 35 sec. falling-ball (5300 centipoises) (360 DP) a salt index of 9.0 and a filtration value of 2800. In the preparation of a similar viscose from identical pulp containing no added cobalt, an aging time of 46 hours at 30° C. was required.

In the preparation of similar viscose from identical pulp containing 0.2 p. p. m. added cobalt the aging requirement was 22 hours at 30° C.

In the preparation of similar viscose from identical pulp containing 1 p. p. m. added cobalt by a similar process except that shredding was for 2 hours at 50° C., no aging time was required, sufficient depolymerization having been accomplished during shredding. Under these same conditions, pulp without added cobalt required an aging time of 24 hours at 30° C.

*Example VIII*

Pulp of 97% alpha, 1550 DP was treated to contain 1 p. p. m. of added cobalt giving it an aging requirement of 5 hours for conversion into rayon type 7.5-6.5 viscose. Identical pulp without the added cobalt had an aging requirement of 42 hours when processed into similar viscose.

*Example IX*

Pulp of 94.9% alpha and 1150 DP was treated to contain added cobalt in amounts of 0, 0.1, 0.5, 1, 2, 5 and 10 p. p. m. When converted to rayon type viscose the aging requirements for these pulps were found to be respectively 30, 17, 10, 6, 3.5, 2.5 and 2 hours at 30° C.

*Example X*

10 A cold caustic refined pulp of 99.3% alpha and 1100 DP was treated to contain 0.2 p. p. m. of added cobalt. When processed into tire cord type viscose the aging requirement was found to be 8 hours at 30° C. With no added cobalt the aging requirement was 24 hours at 30° C.

I claim:

The improvement in the viscose process which comprises aging alkali cellulose prepared from cellulose pulp containing from 83% to 99% of alpha cellulose with the amount of cobalt, based on the bone dry weight of the cellulose pulp, falling within the shaded area and substantially along the ordinate of the alpha cellulose content of the cellulose pulp of the graph of the accompanying drawing.

## References Cited in the file of this patent

## UNITED STATES PATENTS

| 30 | Number    | Name             | Date          |
|----|-----------|------------------|---------------|
|    | 2,542,285 | Mitchell         | Feb. 20, 1951 |
|    | 2,542,492 | Entwistle et al. | Feb. 20, 1951 |

## OTHER REFERENCES

35 "Cellulose and Cellulose Derivatives" (Ott). Published by Interscience Publishers, Inc., N. Y. C., 1943. (Page 744 relied on.)